

Dec. 30, 1924.

1,521,222

M. M. WILCOX

TAPPET

Filed May 31, 1924



Fig. 1



Fig. 2



Fig. 3



Fig. 4



Fig. 5

Inventor

Merrill M. Wilcox

By *Geo. B. Wilcox*

Attorney

## UNITED STATES PATENT OFFICE.

MERRILL M. WILCOX, OF SAGINAW, MICHIGAN.

## TAPPET.

Application filed May 31, 1924. Serial No. 716,979.

*To all whom it may concern:*

Be it known that I, MERRILL M. WILCOX, a citizen of the United States, residing at Saginaw, in the county of Saginaw and 5 State of Michigan, have invented certain new and useful Improvements in Tappets; and I do hereby declare the following to be a full, clear, and exact description of the invention, such as will enable others skilled 10 in the art to which it appertains to make and use the same.

This invention relates to valve tappets and pertains more particularly to certain improvements in the construction of valve 15 tappets such as are commonly used in the engines of automobiles, aeroplanes and the like. My improvement relates more specifically to tappets comprising a tubular body and a cam-contacting head of hardened material, the head formed with an elongated cylindrical shank received within the tubular body and secured thereto by spot welding.

In practice the tubular body is usually of 25 wrought metal such as steel, and the cam-contacting head is of cast iron and has a working face hardened by chilling.

Tappets of this character are described and claimed in my Paent No. 1,470,041, issued October 9, 1923, to which reference 30 may be had.

My present invention has for its objects to increase the wearing qualities and the working life of the tubular body, which in 35 the operation of the engine slides lengthwise in a bearing. After long continued use the tubular bodies or stems of tappets show the first signs of wear at places near the two ends of the stem, doubtless caused 40 by the sidewise thrust of the actuating cam. Extreme hardness is, therefore, essential at areas near the ends of the stem.

Heretofore the spot welding operation has, by reason of heat unavoidably conducted from the weld, reduced the hardness previously imparted to the lower part of the stem. It is a purpose of my invention to enable the stem to retain as nearly as possible the full degree of its initial hardness.

Another object is to provide on the stem or tubular body of the tappet a groove or chamber, the thinner walls of which can be welded to the cylindrical shank of the cam-contacting head in less time than formerly 55 and without so much heat.

This groove also prevents "flashing out" at the edges of the spot weld and thereby does away with the formation of slivers at the edge of the welded area. Such welding 60 slivers or projections are of extreme hardness, being considerably harder than the heat-treated and hardened cylindrical surface of the tappet stem. These extra hard 65 projections on the cylindrical wall of the tappet are a serious disadvantage in manufacture.

Extreme accuracy is required with respect to the diameter of the finished tappet stem, which is usually required to be of uniform diameter throughout its length within tolerances of two tenths of one thousandth of an inch. The tappets must fit in the engine brackets so closely that even when ground to the above degree of accuracy they 75 are inserted in the respective bearings in the tappet bracket of the engine by selection, the tappet best suited for each hole being picked out by trial. If the spot welding is done on the original diameter of the 80 stem without the groove or chamber areas, and the welding flash produces a hardened projection, then in the grinding of the tappet the grinding wheel becomes worn unevenly on account of the extra hard flash 85 weld projections, and after a time it has been found that the tappet diameters are not sufficiently accurate to comply with the requirements. Sometimes around the area in which the flashing has occurred the 90 finished stem diameter will be one-tenth of one thousandth of an inch larger than at any other diameter in its length. Such tappets frequently have to be rejected.

By spot welding in the groove, or in the 95 equivalent chambers, the grinding wheel does not come in contact with a hardened flash projection and consequently is not worn unevenly and will produce uniform grinding for an indefinite length of time. 100

The groove also serves as a gauge to indicate to the operator when the welding contact points have become blunt and require re-sharpening.

5 A still further object of my invention is to provide a circumferential lubricating channel on the tappet stem intermediate the two hardened extremities of the stem.

With the foregoing and certain other objects in view which will appear later in the 10 specifications my invention comprises the devices described and claimed and the equivalents thereof.

In the drawings Fig. 1 is a side view of 15 a tappet embodying my improvement, the hardened areas indicated by stippling and the extent of travel of the tappet by dotted lines.

Fig. 2 is a cross section on the line 2—2 20 of Fig. 1.

Fig. 3 is a side view of a spot welded tubular body indicating the "flashing out" action when the welding groove is not used.

Fig. 4 is a similar view showing the 25 groove and welding spots therein.

Fig. 5 is a side view of a tappet stem showing the spot weld applied to a thin wall formed by milling the spots on the stem instead of on the continuous groove.

30 As is clearly shown in the drawings, 1 is the tappet body and 2 is the head which is usually formed of a separate piece of metal such as cast iron, and hardened either by heat treatment or by chilling. 3 is a flange, 35 the surface of which is preferably hardened to contact with the engine cam 4, as shown in Fig. 1. An elongated axially projecting cylindrical shank 5 is formed on the head 2 and is accurately fitted within the tubular body 1, to which it is secured by spot welding.

In practice the tubular body 1 is independently hardened by heat treatment, the 45 hardness being about seventy points by the scleroscope. To affect the welding without appreciably decreasing the hardness of the lower part of the stem is, as above stated, one of the objects of my improvement.

Referring to Fig. 3, a stem is shown having 50 spot welds applied to its outer surface as has been the practice heretofore. These spots are indicated at 6 and the edges of the spot, as at 7, are usually found to have "flashed out," causing hardened projections 55 or slivers on the outer working surface of the tappet stem, as previously described.

In my present invention I form a groove 60 or chamber 8 by machining the stem 1 before it is hardened, so as to produce a thinner wall  $t$ —see Fig. 2—as compared with the original thickness  $T$ . The spot weld is applied in this groove, as indicated in Fig. 4, instead of through the original thickness  $T$  of the tappet as heretofore.

The groove also prevents the "flashing out" 65 previously noted and in addition serves as a gauge to show the operator when his contact points have become blunt. Heretofore the operator had no means, except by constant inspection, to determine 70 when the contact points required sharpening, but when the welds are produced in the groove 8, as shown in Fig. 4, the edges of the groove itself become a gauge by which the operator is immediately made aware of 75 the fact that the points have become blunt.

Spot welding through the thickness  $T$ , as in Fig. 3, requires more time and more heat than is required to do equally effective welding through the inner wall  $t$ , as indicated in 80 Fig. 4. Thus not only is time saved in the welding operation, but less heat is conducted to the lower part of the hardened tubular stem and consequently its hardness is reduced to a lesser extent than heretofore. 85

In practice the spot welding operation when applied through the full thickness  $T$  of the tappet stem wall as shown in Fig. 3, heats the lower part of the stem to such an extent as to reduce its indicated hardness 90 from about seventy points by the scleroscope to about forty points, but when the weld is applied to the thinner metal  $t$ , forming the wall of groove 8, the lower part 95 of the stem is not heated so much and the hardness is only reduced about one-third as much, or to about sixty points. This enables the lower end of the stem to be kept hard enough to resist wear that could not formerly be resisted.

100 The groove 8 or the equivalent chambered areas also serves as an oil-carrying or lubricating channel to keep the middle part of the length of the stem properly lubricated.

By means above described I have produced a simple and relatively inexpensive, yet strong and durable tappet having the ends of its stem, where the greatest wear occurs, of extreme hardness. The circumferential groove by reducing the time required for welding and the amount of heat required to produce a proper weld, imparts to the completed tappet advantages that have not heretofore been present in two-piece tappets of the class described.

Having thus described my invention, what I claim and desire to secure by Letters Patent is:

1. In a tappet comprising a tubular body and a cam-contacting head formed with an elongated cylindrical shank received within said body, an external circumferential groove formed in said tubular body, the wall of metal of reduced thickness comprising the bottom of said groove spot-welded to said shank.

2. In a tappet comprising a tubular body of hardened metal and a cam-contacting

head formed with an elongated cylindrical shank received within said body, a part of the tubular wall of said body adjacent said shank externally chambered to provide an area of reduced thickness, said wall spot-welded to said shank in said area of reduced thickness, whereby to prevent excessive heat-

ing and consequent reduction of hardness of adjacent parts of said hardened tubular body. 10

In testimony whereof, I affix my signature.

MERRILL M. WILCOX.